

Dec. 2, 1924.

1,517,402

G. CONSTANT ET AL

## PRODUCTION OF IRON AND STEEL BY TREATING DIRECTLY GANGUE FREED ORES

Filed April 11, 1922



INVENTORS

Georges Constant  
and André Bruzac  
By Emile Bönnelycke  
ATTORNEY

Patented Dec. 2, 1924.

## UNITED STATES PATENT OFFICE.

GEORGES CONSTANT AND ANDRÉ BRUZAC, OF PARIS, FRANCE.

PRODUCTION OF IRON AND STEEL BY TREATING DIRECTLY GANGUE-FREED ORES.

Application filed April 11, 1922. Serial No. 551,554.

*To all whom it may concern:*

Be it known that we, GEORGES CONSTANT, a citizen of the Republic of France, and a resident of Paris, France (post-office address 5 1 Rue Drouot), and ANDRÉ BRUZAC, a citizen of the Republic of France, and a resident of Paris, France (post-office address 1 Rue Drouot), have invented new and useful Improvements in the Production of Iron 10 and Steel by Treating Directly Gangue-Freed Ores, which improvements are fully set forth in the following specification.

The object of our invention is to provide a method or process for making iron or steel, 15 consisting in treating the ores freed from all their gangue, in such a manner as to prevent the formation of any slags which would make it impossible to use the melting or smelting furnace.

20 The process which is the object of our invention is characterized by the following operations:

A. Ore crushing.

B. Washing of the crushed ore in order 25 to remove all or part of the gangue. In certain cases this removal of the gangue may be effected magnetically.

C. Drying of the ore freed from its 30 gangue by any process (ventilation or mechanical stirring may even be used).

D. Reduction of the ore in a closed vessel by any reducing or deoxidizing gas (poor 35 gas, water gas, etc.) or any other suitable reducer; this reduction is effected very promptly due to the fine molecular state of the ore.

E. The ore having been reduced, direct 40 passage of the metal from the reservoir or tank to the reducing apparatus, without any contact, or with as short a contact as possible, with air in a Martin, Siemens or other smelting furnace.

45 Before charging, a non-oxydizing atmosphere may be created in the furnace by keeping the said furnace only partly lighted or by any other means.

F. Smelting of the metal by ordinary 50 processes, with the addition of a small quantity of corrective (lime or other substance, according to requirements).

The melted metal will be, according to the reducer used, either iron or steel and, by means of the well known additions, it will be easy to obtain such steel as desired.

55 Similarly, cast-iron may be obtained. Whenever any slight oxydizing of the metal

takes place a corrective agent will have to be used.

Also after crushing, the ore may be reduced and then freed from its gangue either 60 as indicated in paragraph B above, or by any other means . . . such oxydizing as may result from this method of operation should be corrected in the melting furnace.

In order to make the invention more 65 clearly understood we have appended hereto a drawing, the single figure of which represents diagrammatically a practical embodiment of the invention.

In carrying out the process, the ore washed 70 at the mine should reach the crushing mill practically free from gangue.

It can be dried by means of the waste heat of the mill and then passed on to the reduction chamber where the first operation 75 will be to make it lose, if necessary, the remainder of its moisture and the small quantity of carbonic acid it may yet contain.

This result will be obtained by drawing 80 the residuary gases left in the smelting furnace (reverberatory furnace), from the latter through valve D and thence through the mass of ore in the reducing chamber.

The reducing chamber A must be hermetically closed at the top by a flap cover 85 or any other cover forming a joint.

The bottom closure will be a device such as the one usual with a blast furnace throat but any other sort of closure may be used such as a movable slide worked from outside, or a sort of jack having a suitable bearing point and supporting a conical plug or obturator, such jack being worked from outside by means of, say, a worm.

The casing of the reducing chamber and 90 the throat B extending below should be perfectly tight.

During reduction, the bottom of the throat should be closed by a solid plug which will be replaced by a movable sleeve M at the 95 time when the reduction chamber is emptied and before removal of the cone which serves as its bottom closure.

Such sleeve must be luted at both ends in order to make a joint with the throat and 100 with the reverberatory furnace; it will rest on a metal part or member N cooled by an internal water jacket.

Tightness of the reducing chamber at the 110 top and also of its casting, as well as of the throat, being achieved, it will be easy to cause the gaseous reducing agent to expand

and make its way through the mass of ore, and thus obtain an intimate and absolute contact of the gas and of the ore, conducive to reduction.

5 Similarly, it is possible, in certain cases, to force the reducing gas under pressure into the mass of ore.

The reducing gas is drawn through the inlet pipe and its valve C from a suitable 10 source of supply, due to the suction action of a pump or fan J, into the reduction chamber A, and is discharged from the latter through a pipe E into a dust box F. From 15 this box, it passes through a cooler G, where its temperature is lowered, and thence through a meter I into the fan casing; a valve H being interposed between the cooler and the meter.

A pipe L, connected to the fan or pump J, 20 is utilized to evacuate such gases as might remain in throat D before unplugging the same to position sleeve M.

It will be easy to make sure, by means of 25 the meter of each reduction chamber, that the quantity of gas necessary to reduce the contained ore has passed through the chamber, and the fact should be ascertained periodically, by using an automatic recording analyser K or by any other means, that the 30 carbonic oxid of the reducer gas has been transformed into carbonic acid.

A pyrometer, indicating the temperature at which the reduction is made and the time 35 consumed in the operation will give the carburetion degree of the iron.

If it is iron that is to be made, very slightly carbureted steel is made and then this steel is decarburized by the corresponding 40 quantity of  $Fe_2O_3$ .

It is therefore steel that is sent from the reducing chamber into the smelting furnace.

The number and size of the reducing chambers depend upon the reduction time and tonnage of the smelting furnace.

45 The work of such chambers is arranged in successive stages so as not to cause any loss of time at the smelting furnace.

They can be made of cast iron or of steel and should be faced both inside and outside with refractory material suitably supported and reinforced.

Downwardly inclined holes will be arranged for the inlet of the reducing gas into the lower part.

The metallic casing must be tight, as 55 aforesaid; it should be lined on the inside with refractory material and the reducer gas should be permitted to circulate between this lining and the conical lower portion of the reducing chamber, so as to have access 60 to all the inclined inlet holes just mentioned.

Rigidly mounted on a suitable metallic structure, they will overhang the smelting furnace into which they will easily empty 65 on the side opposite the tap hole.

We claim as our invention:

1. A process of making iron or steel, comprising the steps of subjecting the gangue-free ore, in an air-tight reduction chamber, to the action of carbonic oxid which is being 70 constantly renewed, bringing the ore and carbonic oxid to a predetermined temperature which is below the point where the ore becomes pasty and maintaining such temperature for a definite period of time which 75 is a function of the temperature, thereby to obtain complete reduction and carburetion of the metal and its consequent conversion into steel in said chamber; substantially as described.

2. A process of making iron or steel, comprising the steps of subjecting the gangue-free ore, in an air-tight reduction chamber, to the action of carbonic oxid which is being constantly renewed, bringing the ore 85 and carbonic oxid to a predetermined temperature which is below the point where the ore becomes pasty and maintaining such temperature for a definite period of time to obtain completely reduced and carbureted 90 metal in the reduction chamber in the form of pieces of steel sponge, and then immediately smelting said pieces to fuse them and separate out any impurities which may still remain; substantially as described. 95

In testimony whereof we have signed this specification in the presence of a subscribing witness.

GEORGES CONSTANT.  
ANDRÉ BRUZAC.

Witness:

CHARLES LEÓN LOISÉ.